

C. ROBINSON.

PROCESS FOR DESULFURIZING AND AGGLOMERATING ORES.

APPLICATION FILED JUNE 27, 1908.

926,289.

Patented June 29, 1909.

3 SHEETS—SHEET 1.

Fig. 1.



Witnesses:

James Ober  
William F. Muller

Inventor  
Cyrus Robinson  
By his Attorney  
Oscar M. Bird

C. ROBINSON.

PROCESS FOR DESULFURIZING AND AGGLOMERATING ORES.

APPLICATION FILED JUNE 27, 1908.

926,289.

Patented June 29, 1909.

3 SHEETS—SHEET 2.



Witnesses:

James O. O.  
William F. Muller.

Inventor

By his Attorney Cyrus Robinson  
Warren Dink

C. ROBINSON.

PROCESS FOR DESULFURIZING AND AGGLOMERATING ORES.

APPLICATION FILED JUNE 27, 1908.

926,289.

Patented June 29, 1909.

3 SHEETS—SHEET 3.

Fig. 3.



Fig. 4.



Witnesses:

James Ober

William T. Muller

Inventor  
Cyrus Robinson  
By his Attorney  
Wm. A. Dier

# UNITED STATES PATENT OFFICE.

CYRUS ROBINSON, OF MOUNT VERNON, NEW YORK.

## PROCESS FOR DESULFURIZING AND AGGLOMERATING ORES.

No. 926,289.

Specification of Letters Patent.

Patented June 29, 1909.

Application filed June 27, 1908. Serial No. 440,761.

*To all whom it may concern:*

Be it known that I, CYRUS ROBINSON, a subject of Great Britain, residing at Mount Vernon, in the county of Westchester and 5 State of New York, United States of America, have invented a new and useful Process for Desulfurizing and Agglomerating Ores, of which the following is a specification.

My invention relates to improvements in 10 processes for desulfurizing and agglomerating sulfid and other ores, and among the objects of my improvements are, (1), to provide a process by which ores can be desulfurized and agglomerated continuously; (2), to accomplish this without the use of extraneous 15 fuel or heat after the inception of the combustion, and also without the use of any reagents; (3), to shorten the period of operation; (4), to produce a sinter which can be 20 smelted in the blast or other furnace without briquetting or any intermediate treatment whatever; (5), to collect the sulfur gases in such concentrated form that they may be readily converted into sulfuric acid.

25 My process is designed for desulfurizing and agglomerating any sulfid ores or a mixture of sulfid, fine ore and fluxes, whereby a product will be discharged in condition for smelting without further treatment. In all 30 other processes known to me, it is necessary to use extraneous fuel for each charge to be treated, or where the process is continuous by the continuous application of extraneous heat. This consumption of fuel, not only 35 makes such processes expensive by comparison, but involves with many roasters, the installation of apparatus for the manufacture of gas or charcoal. In my process, after it is once put in operation the roasting and ag- 40 glomerating may be continued indefinitely without the use of extraneous fuel where the sulfur is sufficiently high to perpetuate the combustion, and if it is desired to roast and agglomerate ores containing too little sulfur 45 for such result, I mix with the ore to be treated, coke fines or other fuel to assist in the roasting and agglomerating. Again in the methods referred to, it has been found that the results are very imperfect without 50 the use of some reagent, such as oxid of lime, to prevent the ore forming into masses or cakes before a satisfactory desulfurization has occurred. The objections above pointed out, I overcome by my improved process,

which as will appear below is continuous in 55 operation, makes use of no reagent, and delivers the desulfurized ore in an agglomerate form and a partially fused condition, avoiding the necessity of "briquetting" and effecting a saving of fuel in smelting.

60 I attain the above mentioned objects by the process hereinafter described.

In the accompanying drawings, I have 65 illustrated a form of apparatus which is adapted for carrying out my process.

Figure 1, is a vertical sectional view of my apparatus on the line X—X of Fig. 2. Fig. 2, is a vertical sectional view at right angles to Fig. 1. Fig. 3 is a horizontal sectional view through the air chamber. Fig. 4 is a 70 detailed view of a surface of a roll.

In the drawings 1 represents the vertical 75 rectangular body portion or roasting chamber supported on bearings 15, and surrounded by an ore hopper 2. I construct 80 my roasting chamber of a limited depth so that a comparatively thin stream of ore is passed through the same. This is preferred, as it is in the treatment of large quantities of ore under blast that the formation of slag in 85 the center and the failure to sinter at the top takes place. This chamber 1 is surrounded at the base by a hood 3, extending below the same and covering a pair of toothed rolls 8. Surrounding said roasting chamber at a suitable height is a chamber 4, which is connected 90 with the air blast at the inlet 10. Access by the air to the inside of said roasting chamber is gained through apertured plates or grates 5. At a suitable distance above said chamber 4 is another chamber 6 surrounding said body and provided with an outlet 11 for the discharge of the gases, which pass into said chamber from the roasting chamber through the perforated plates 12. The gases which 95 find their way downward are collected by the hood 3 and rise through the flue 15 to either the outlet 11 or 17 according to the arrangement of the dampers 18 and 16.

The rolls 8 are located below the greater 100 sides of the roasting chamber in such relative positions that their teeth 9 and 19 will engage the descending desulfurized and agglomerated ore. These rolls are driven by any suitable mechanism and being rotated downwardly 105 toward each other at a predetermined speed regulate and assist the flow of the descending material through the chamber. Some of the

teeth (19) I construct deeper than the others for the purpose of breaking the agglomerated material into sinters of suitable sizes.

The process is as follows:—Chamber 1 is filled with some material such as refuse ore up to a point approximately level with the top of grate 5. On top of this bed of material a fire of wood, charcoal, or any combustible material, is lighted. A light blast is then turned on through air inlet 10 aiding the combustion of the fuel. Ore is then fed into the machine through hopper 2 until the hopper is filled. Combustion is then started in the bottom layer of ore and mounts upward to a point a short distance below the smoke outlet. As soon as sulfur fumes are noted at the smoke outlet, the rolls 8 are set in motion and the material is gradually and regularly fed through the roasting chamber. The air blast is maintained at such a pressure as to create a temperature which at its maximum will slightly fuse the ore and cause its agglomeration. When this stage is passed most of the desulfurization has taken place but the process of desulfurization continues so long as the material is in the chamber. The rolls 8 can be adjusted laterally by means of adjusting screws, as shown, so that the agglomerated and roasted product can be discharged in blocks of convenient size for handling and treatment in the furnace. The revolution of the rolls is maintained at such a speed that the ore while passing through the roasting chamber remains therein the time required to effect its desulfurization, and so that one continuous stream of agglomerated ore is discharged from the roasting chamber so long as the ore supply and air blast supply are maintained.

In some cases it has been found that the ore has a tendency to incrust upon the sides of the roasting chamber. To prevent this incrustation, I provide an annular trough 6 and a series of perforations 20 leading therefrom into the roasting chamber. A fluid mixture of graphite and soft soap or other suitable material being placed in the trough passes through the said perforations and down the inside of the walls of the roasting chamber thus preventing the incrustation mentioned, at the same time cooling the walls.

Other forms of apparatus may also be used, and I therefore specifically state that I do not wish to be limited to the form here-with illustrated.

I claim:

1. The method of continuously desulfurizing ores, which consists in maintaining a zone of heat in a passing stream of ores without the use of extraneous fuel.
2. The method of continuously desulfurizing and agglomerating ores, which consists in passing said ores through a narrow chamber and subjecting them to the action of heat

in an oxidizing atmosphere in said chamber without the use of extraneous fuel.

3. The method of continuously desulfurizing ores, which consists in raising the temperature of successive layers of said ores to the required point without the use of extraneous fuel.

4. The method of continuously desulfurizing ores, which consists in continuously subjecting successive layers of moving ore to the action of heat in an oxidizing atmosphere without the use of extraneous fuel.

5. The method of desulfurizing ores, which consists in mixing a fuel with said ores and passing the same through a zone of heat, whereby combustion is continuously maintained therein without recourse to extraneous heat.

6. The method of continuously desulfurizing ores, which consists in maintaining a current of air through a given portion of a stream of moving ore whereby combustion is maintained therein continuously without the use of extraneous fuel.

7. The method of continuously desulfurizing and agglomerating ores, which consists in maintaining a zone of heat in a passing stream of ores by means of the combustive properties in said ores without the use of extraneous fuel or heat.

8. The method of continuously desulfurizing and agglomerating ores, which consists in maintaining a zone of heat in a passing stream of ores solely by means of the combustive properties in said ores and passing a current of air through said zone.

9. The process of treating ores containing combustible elements, which consists in starting combustion in a stream of the ore and thereafter maintaining combustion in said stream without the use of extraneous fuel.

10. The process of treating ores containing combustible elements, which consists in feeding the ores through a zone of combustion, in initially applying extraneous heat to start combustion in the ore passing through said zone and in thereafter maintaining combustion in said stream without the use of extraneous heat.

11. The improvement in the art of treating ores so as to produce desulfurization and agglomeration which consists in igniting a stream of ore in a chamber, in feeding said stream of ore regularly through said chamber, in introducing a current of air into said moving stream of ore at a definite point between the inlet and outlet of said chamber, and in educating said current of air with the products of combustion after passing through the ore from a definite point between the air and ore inlets and also at a definite point beyond the air inlet.

12. The improvement in the art of treating ores so as to produce desulfurization and ag-

glomeration which consists in igniting a stream of ore in a chamber, in feeding said stream of ore regularly through said chamber, in introducing a current of air into said moving stream of ore at a definite point between the inlet and outlet of said chamber and educing a part of said current of air with the products of combustion at a definite point between the air and ore inlets so as to produce a gas with a high percentage of sulfur for use in the arts.

13. The improvement in the art of treating ores so as to produce desulfurization which consists in maintaining a zone of continuous heat in a passing stream of ores without the use of extraneous fuel or heat.

14. The improvement in the art of treating ores so as to produce agglomeration which

consists in maintaining a zone of continuous heat in a passing stream of ores without the use of extraneous fuel or heat.

15. The improvement in the art of treating ores so as to produce desulfurization and agglomeration, which consists in igniting a stream of ore in a chamber, in feeding said stream of ore regularly through said chamber, in maintaining a current of air through a definite zone of said moving stream of ore in said chamber, and in treating the inner walls of said chamber so as to prevent the incrustation of the ore thereon.

CYRUS ROBINSON.

Witnesses:

BENJ. PRINCE,  
FRANCIS RISK.